

No. 710,496.

Patented Oct. 7, 1902.

S. T. MUFFLY.

PROCESS OF TREATING ORES.

(Application filed Sept. 20, 1901.)

(No Model.)

3 Sheets—Sheet 1.



FIG. 1.

WITNESSES

*F. A. Stewart*  
*F. F. Teller*

INVENTOR

BY *Sidney T. Muffly*

*John J. Patten* ATTORNEYS

No. 710,496.

Patented Oct. 7, 1902.

S. T. MUFFLY.

PROCESS OF TREATING ORES.

(Application filed Sept. 20, 1901.)

(No Model.)

3 Sheets—Sheet 2



WITNESSES

F. A. Stewart  
M. G. O. Teller

BY

INVENTOR  
Sidney T. Muffly

ATTORNEYS  
John Peter

No. 710,496.

Patented Oct. 7, 1902.

S. T. MUFFLY.

PROCESS OF TREATING ORES.

(Application filed Sept. 20, 1901.)

(No Model.)

3 Sheets—Sheet 3



WITNESSES

J. A. Stuart  
F. F. Eller

BY

Sidney T. Muffly, INVENTOR

S. T. Muffly  
ATTORNEYS

# UNITED STATES PATENT OFFICE.

SIDNEY THEODORE MUFFLY, OF BOWDRE, GEORGIA, ASSIGNOR OF ONE-HALF TO RUNYON PYATT, OF NEW YORK, N. Y.

## PROCESS OF TREATING ORES.

SPECIFICATION forming part of Letters Patent No. 710,496, dated October 7, 1902.

Application filed September 20, 1901. Serial No. 75,800. (No specimens.)

To all whom it may concern:

Be it known that I, SIDNEY THEODORE MUFFLY, a citizen of the United States, residing at Bowdre, in the county of Hall and 5 State of Georgia, have invented certain new and useful Improvements in Processes of Treating Ores, of which the following is a full and complete specification, such as will enable those skilled in the art to which it app- 10 pertains to make and use the same.

This invention relates particularly to processes for the extraction of gold and silver from ores, concentrates, slimes, and tailings by the use of cyanid of potassium or other 15 chemicals; and it has for its object to provide such a process or method as will effectually and economically supply oxygen to the ores during treatment, create and maintain a requisite and constant temperature, supply 20 the solvent effectively as desired, and in general bring about a more perfect and considerably more rapid leaching of the gold or silver.

With these and other objects in view my 25 invention consists in the process or method hereinafter fully described and claimed.

In carrying out my newly-invented process I may construct the necessary apparatus or plant in any desired manner, according to the 30 amount or character of ores to be treated. The apparatus best adapted to the practice of my process is one which I have invented and have made the subject of an application for patent filed in the United States Patent 35 Office of even date herewith—viz., on the 20th day of September, 1901, Serial No. 75,799—and for the full and thorough comprehension of my process and the mode of carrying it into effect I will first describe this said ap- 40 paratus and then proceed to define the mode of operation of my process.

In the accompanying drawings, forming part of the specification, in which like letters of reference designate corresponding parts, 45 Figure 1 is a side elevation, partially in section, showing an apparatus embodying my invention aforesaid. Fig. 2 is a perspective elevation of the cylinder and the gearing thereof. Fig. 3 is a partially-broken central 50 vertical section of the cylinder and its inlet and outlet pipes. Fig. 4 is a detail view of

the closure device of the cylinder. Figs. 5, 6, and 7 are details, respectively, of the filter-plate, the cover-plate, and the securing device forming part of the said closure. 55

In the practice of my invention aforesaid I construct a cylinder A of any suitable form and material and line it interiorly with a plurality of plates closely adjacent liner-plates B. Within the cylinder A, I secure a 60 plurality of longitudinal strips or baffles C at suitable distance apart. In any suitable portion of the circumference of the cylinder, and preferably near the end thereof, I form an opening for the insertion of the ores and 65 chemicals, over which I secure the feed-hole casing D, the flange D' of which extends over the feed-opening in the cylinder and is tightly fastened. Within the casing D is formed a ledge or shoulder D<sup>2</sup>, on which rests a filter- 70 device E, which consists of a metallic plate centrally open and a similar and smaller supplemental plate E', between which plates are secured layers of cotton-duck E<sup>2</sup> and cocoa matting E<sup>3</sup>, both plates and the said layers 75 being secured together by means of bolts. Above the filter-plate E is secured the cover F, which rests within and upon the upper edge of the casing D and projects thereover. In lugs D<sup>3</sup>, at either side of the casing D, is 80 pivoted a segmental cross-head G, through which extends a hand-screw G', the lower end of which bears upon the cover-plate F, so as to clamp the same in position upon the feed-hole casing. The filter-plate E and the cover- 85 plate F may be employed together, as shown in Fig. 4, or the cover-plate and the filter may be used alternately and separately. Upon either end of the cylinder I secure hollow axles H, provided with integral flanges or plates H', 90 by which they are bolted to the ends or heads A' of the cylinder. The axles rest in suitable bearings I' upon a framework or uprights I of any desired or approved form. At the end of the said axles is formed a stuffing-box H<sup>2</sup>, 95 in which is inserted the end of an inlet-pipe J or an outlet-pipe J'. Within the cylinder, in communication with the hollow axles H, are small chambers K and K', which communicate with the interior of the cylinder only 100 through valves L and L', pivoted at L<sup>2</sup>. The valves of the inlet-chamber K swing out-

wardly to permit the entrance of air into the cylinder, and the valves L' of the outlet-chamber K' swing inwardly to permit the exit of the hydrocyanic-acid fumes within the cylinder. Any suitable means may be employed for limiting the swing of the valves. In the drawings I have shown weak springs M and M' for this purpose. The spring M is secured upon the outside of the chamber K and projects around the pivot L<sup>2</sup>. The spring M' is secured within the chamber K' and bears lightly against the valves L' upon their inner faces. It will be manifest that any suitable valves may be employed.

15 Upon the outside of one end of the cylinder A is secured a circumferentially-extending spur-gear N, attached to the said cylinder in any desired manner and meshing with a pinion O, connected to a pulley P, supported upon a shaft Q, suitably journaled in the framework I. In the end of the cylinder are inserted a plurality of drainage-valves R.

The inlet-pipe J projects from an air blast or blower S, operated by any suitable power, 25 from which air is injected through the said inlet-pipe J, formed into a worm or plurality of coils J<sup>2</sup>, and this portion of the pipe is continued in the hot-air box or casing of a furnace T, through which the said pipe J passes, 30 the furnace being generally part of the plant which operates the machines, or it may be separate therefrom, if desired.

Between the furnace T and the cylinder A there is connected to the pipe J by a T-coupling J<sup>3</sup> a pipe U, leading downwardly from a tank V, which contains cyanid of potassium in solution, preferably a one-half-of-one-per-cent. solution. The elevation of the tank V is to give sufficient force of flow to the fluid 35 solution. The pipe U beneath the tank is provided with a stop-cock or regulating-valve W, and the pipe J rearwardly of the coupling J<sup>3</sup> is provided with a similar regulating-valve W'. Above the coupling J<sup>3</sup> is an ejector Y.

40 The operation of my newly-invented process is as follows: The ores and a small portion of a weak solution (preferably a one-quarter-of-one-per-cent. solution) of cyanid of potassium and only sufficient in amount to saturate the ores are inserted through the feed-hole of the cylinder and the latter closed by means of the cover-plate F and the clamping-screw G'. Power is then applied to the pulley P to rotate the cylinder, and the effective 45 leaching of the ores then commences. As the operation continues air of the most efficient temperature and a fresh solution of the same or any other desired strength (according to the character of the ore under treatment) is forced through the inlet-pipe J and valves L into the cylinder in the form of a spray. Air 50 may be forced in alone either hot or cold and its amount and force governed by the regulating-valve W', and by turning on the regulating-valve W the cyanid solution enters the air-inlet pipe J and is injected with the air into the cylinder. The amount of cyanid in-

roduced is regulated by the valve W and also in part by the air-pressure valve W'. When the apparatus is employed exactly as 70 shown in the drawings, a combination of hot air and cyanid-solution spray will be injected into the cylinder under considerable pressure. In practice I prefer to heat the air in the treatment of oxidized ores to about 100° 75 Fahrenheit, and with other ores the temperature will be higher or lower, according to the character of the ores or the elements they contain. This injection of air and cyanid, especially coincidently with the revolution of 80 the cylinder A, serves a plurality of purposes. It provides a more effectual and economical supply of oxygen. It creates and maintains the most effective and the most constant temperature. It instantaneously adds fresh 85 cyanid of potassium or other solvent in the form of spray continuously. It forces the oxygen and also the solution into and between all the parts of the ore charge during any special time or during the entire time, according to 90 the character of the ores operated upon. It supplies oxygen to replace that element as rapidly as it separates from the cyanogen compound to enter into new molecular combination with gold, silver, and potassium. It 95 regenerates or strengthens the solution with a constant supply of the solvent compound, thereby preventing chemical inertia by replacing cyanogen which has combined with hydrogen liberated in the passing over of oxygen to form the new compounds—auro-potassic 100 cyanid, argento-potassic cyanid, and potassic hydrate. Moreover, a systematic agitation is produced in which the ore is carried up by the baffles and falls by its gravity back 105 through the warm currents of air and spray of solution, and in this systematic agitation, besides supplying oxygen to replace that element as it is needed in the cyanogen compounds, another purpose is also served of removing films of insoluble basic oxids from the 110 surface of coarse gold, rendering it more immediately amenable to the chemical treatment. My improved method also accomplishes the 115 expulsion, through the outlet-chamber K past the valve L' and through the outlet-pipe J' to a safe distance outside the building, of the 120 poisonous hydrocyanic fumes generated from the excess of hydrogen and cyanogen liberated by the combination of the oxygen with gold, silver, and potassium. The agitation 125 of the ores and chemicals by the strips or baffles C also breaks up and thoroughly disintegrates the vitrified lumps occurring in ores or concentrates from imperfect roasting 130 and likewise wears away impenetrable masses of slime, thereby bringing the gold and silver 135 more readily in contact with the cyanid of potassium or other chemicals. Coarse gold, which is oftentimes discharged from leaching-cylinders with the tailings after treatment, is in this device worked upon by baffles until the chemical extraction becomes nearly 140 perfect. From the continuous regenerating

or strengthening of the solution with a fresh supply of the solvent I replace cyanogen which has combined with liberated hydrogen and potassium cyanogen that have combined with gold and silver in the reaction forming double cyanid as follows:



10 and



15 The agitation of the ores and wearing away of films of insoluble basic oxids from the surface of coarse gold render it more immediately amenable to the cyanid treatment. Any hydrocyanic acid fumes which may be present are forced by the supplied air-current entering through the inlet-pipe J outwardly into the outlet-chamber and outlet-pipe to a point out of the building. Not only is the element thus removed, but, moreover, a continuous 20 current of air thus circulates longitudinally of the cylinder, and the ores as they are tumbled by the baffles E of the cylinder pass through this air and receive a spray or bath of the oxygen and solvent cyanogen compound.

30 I do not desire to confine myself to every step or detail of my process as herein described, as it is apparent that changes therein and modifications thereof may be made 35 without departing from the spirit of my in-

vention or sacrificing its advantages, and I reserve the right to make all such alterations therein as fairly come within the scope of my invention.

Having thus fully described my invention, 40 what I claim as new, and desire to secure by Letters Patent, is—

1. The process of treating ores which consists in saturating the said ores with a chemical solvent, revolving the ores and solvent, 45 agitating and breaking up the ores, injecting a current of heated air under pressure charged with fresh solvent in the form of a spray at one point to the ore charge, circulating the said spray through the ore charge 50 axially of its revolution and agitation, and carrying off liberated elements and fumes at a point opposite to the injection of the spray.

2. The process of treating ores herein described which consists in injecting into said 55 ores, as they are agitated and elevated and allowed to fall by gravity in a closed chamber, a chemical solution in the form of a spray together with hot air under pressure, and allowing the elements and fumes freed by this 60 operation to escape from said chamber, substantially as described.

In testimony that I claim the foregoing as my invention I have signed my name, in presence of the subscribing witnesses, this 13th 65 day of September, 1901.

SIDNEY THEODORE MUFFLY.

Witnesses:

B. H. ABBOTT,  
A. G. DORSEY.